

1

2,810,684

## DIAPHRAGM FOR MANGANESE ELECTROWINNING

Robert H. Cromwell, East Orange, N. J., and William A. Parsons, Knoxville, Tenn., assignors, by mesne assignments, to Foote Mineral Company, Philadelphia, Pa., a corporation of Pennsylvania

No Drawing. Application October 21, 1954,  
Serial No. 463,826

5 Claims. (Cl. 204—105)

This invention relates to electrowinning manganese, and more particularly to the use in an electrolytic manganese process of a new and improved diaphragm by means of which notable economies in operation of the process are attained. This application is a continuation-in-part of our copending application Serial No. 223,168, filed April 26, 1951, now abandoned.

In the commercial electrowinning of manganese, a direct electric current is passed between an anode and a cathode through a purified manganese sulfate-ammonium sulfate electrolyte. The electrolyte adjacent the anode (the anolyte) is of markedly different composition than the electrolyte adjacent the cathode (the catholyte). Both electrolytes generally contain from 120 to 200 grams per liter of ammonium sulfate; but the catholyte is distinctly alkaline at a pH of about 8 to 9 and contains from 30 to 40 grams per liter of manganese (as manganeseous sulfate), whereas the anolyte is strongly acid with a pH in the range from 0.8 to 1.4 and contains from 12 to 16 grams per liter of manganese.

A diaphragm must be employed in the electrolytic cell to separate the anolyte from the catholyte. The diaphragm must provide for effective physical separation of the anolyte from the catholyte so that no excess diffusion of one into the other takes place. However, the process involves feeding strong electrolyte high in manganese into the catholyte compartment of the cell, where it becomes depleted in manganese as the metal is deposited on the cathode, and correspondingly withdrawing anolyte from the anolyte compartment, where it becomes enriched in sulfuric acid in proportion to the amount of manganese deposited. Consequently the diaphragm must be sufficiently permeable to the electrolyte so as to permit it to flow from the catholyte compartment into the anolyte compartment at essentially the same rate as fresh electrolyte is fed into the catholyte. Moreover the diaphragm must permit the flow of the electric current through it without introducing a very high electrical resistance into the current path. The diaphragm must also be capable of withstanding the severe chemical environment to which it is subjected in normal use. It must withstand the attack of an alkaline ammonium hydroxide catholyte on one side while it is simultaneously exposed on the other side to a strongly acidic sulfuric acid anolyte. Moreover, some of the manganese salts present in the electrolyte are unavoidably converted to manganese dioxide and to permanganates, and these compounds subject the diaphragm to severe oxidizing influences.

Prior to the present invention, and since the beginning of the commercial art of manganese electrowinning, a heavy cotton canvas or duck has been the only satisfactory material of which to make the diaphragm. The most satisfactory cotton fabric diaphragm material has been heavy duck, weighing about 21 ounces per square yard, woven of 3-ply strands with 29 filling strands and 36 warp strands per square inch. The life of such a diaphragm is only about six to eight weeks in normal service. At the end of such period of time, the pores of the fabric have be-

2

come so plugged with a deposit of salts from the electrolyte that the diaphragm is no longer adequately permeable. Moreover, it has become so weakened physically by the chemical action of the electrolyte that it is usually impractical, and in many cases even impossible, to clean it. The cost of labor and materials for replacing these heavy cotton duck diaphragms is of course very high, being, for example, upwards of \$25,000 per year in a plant operating, say, seventy cells with twenty diaphragm chambers per cell.

It has long been recognized that important economies could be achieved in the electrolytic manganese process were it possible to provide a diaphragm which would not need replacement at the end of each cell cycle of six to eight weeks or thereabouts; and much effort has been devoted to a search for a satisfactory diaphragm to replace cotton duck. Early attempts were made to make diaphragms of wool, which is highly acid resistant, but the wool is dissolved by the alkaline catholyte and so is less satisfactory than cotton. The various rayons, including the viscose, acetate and cuprammonium products, proved unsatisfactory because of low wet strength and inability to resist gradual stretching with objectionable increase in permeability. The acetate rayons, moreover, were attacked by prolonged exposure to the acid anolyte, and all of the rayons are weakened by the chemical attack of the electrolyte. Nylon proved entirely unsatisfactory because of its solubility in the acid anolyte. A diaphragm of woven glass fiber cloth seemed promising, but it proved impossible to weave a cloth of glass fibers having the requisite tightness of weave and corresponding low but definite permeability. Moreover, the glass fibers were slowly attacked by the alkaline catholyte, leading to the contamination of the electrolyte with dissolved silica which has been found to be a most objectionable impurity in the electrolyte solution. "Vinyon"—a fabric woven of fibers of the copolymer of vinyl chloride and vinyl acetate—seemed to be quite resistant chemically to the electrolyte, but diaphragms made of it stretched so much under their own weight after a period of immersion in the electrolyte and their permeability so increased that they ceased to provide effective separation of the catholyte from the anolyte. Micropore rubber, a sheeted foamed rubber having numerous minute pores extending through it was tried but was found to stretch objectionably unless supported on a metal backing. The introduction of a metal-backed product into the electrolyte was most objectionable, but might have been tolerated had it not been for other defects of the rubber. One such defect was a lack of uniformity in its permeability. Another was that it becomes oxidized and embrittled by the manganese dioxide and permanganates which form in the electrolyte, and the sulfur, accelerators, and other substances present in the rubber are oxidized to thionates and other objectionable contaminants in the electrolyte. For these reasons, micropore rubber and other rubberized diaphragm materials are impractical. Asbestos fiber diaphragms proved to be mechanically weak and heavy, and additionally were subject to the same disadvantage as glass fiber diaphragms—silicon dissolves in the alkaline catholyte and leads to objectionable contamination of the solution. Porous ceramic diaphragms cannot be employed because when made sufficiently permeable they are too fragile for practical commercial use. Porous carbon diaphragms, while chemically satisfactory, are objectionable because of the bipolar effects they produce in the cell owing to their electrical conductivity. Attempts have been made to make diaphragms of electrostatically perforated films and sheets of various plastic materials, including sheets of polyvinyl chloride, paper coated with pyroxylin, etc., but it proved impossible to control the perforations to give the requisite permeability without so much non-

uniformity as to result in excessive permeability over some areas of the diaphragm sheet.

Thus, although many efforts have been made and numerous materials had been tried to find a better diaphragm, cotton duck remained, for many years, the most practical and only commercially satisfactory diaphragm material available to the art. The present invention provides the first acceptable substitute for a cotton diaphragm that has been developed, and the first which has made it possible to operate more economically than with cotton diaphragms. Strangely enough, considering the large number of materials that have proved unsatisfactory, we have now found that eminently satisfactory diaphragms can be made from fibers of either linear homopolymers of acrylonitrile or polytetrafluoroethylene.

The suitability of diaphragms made of fabrics woven from fibers of these particular synthetic resinous materials resides not simply in the fact that such fibers are resistant to chemical attack by the electrolytes, or even simply in the fact that such fabrics possess high wet strength and other good physical properties. These properties are of course important, but a major contributing factor to the success of the invention lies in the fact that these fibers lend themselves to the construction of a closely woven fabric which possesses, and which retains over prolonged periods of time and through repeated cycles of use in the electrolytic cells, a satisfactory permeability to the electrolytes—a permeability which is low enough to prevent objectionable intermixing of anolyte and catholyte, and yet which is high enough to allow the required seepage of catholyte into the anolyte compartment as electrodeposition of manganese proceeds. The invention, therefore, in addition to being characterized by the use of a diaphragm made of a fabric woven of one of the above-mentioned synthetic fibers, is further characterized by the fact that such fabric is closely woven and has a maximum permeability measured by the flow of catholyte therethrough into the anolyte of not more than about 25 cubic centimeters per square foot per minute under a hydrostatic head of catholyte with respect to anolyte of  $\frac{1}{2}$  inch, and by the ability of such fabric to resist physical deformation and any significant change (especially any increase) in its permeability characteristics during or in consequence of prolonged exposure to the electrolyte.

The minimum permissible permeability of the diaphragm material is determined primarily by economic considerations. Theoretically, the diaphragm can be used if it possesses any degree of permeability. As a practical matter, however, if the permeability is too low, the seepage of catholyte through it will be too slow to meet the demands of an economic rate of electrodeposition. Also, if the permeability is very small, the diaphragm will have the effect of imposing a correspondingly high resistance in the current path between anode and cathode, and as a result the cell voltage drop due to the presence of the diaphragm will be so high as to result in uneconomically high power consumption. Accordingly, the permeability of the diaphragm, in terms of the flow of catholyte therethrough into the anolyte, should be at least about 20 cubic centimeters per square foot per minute under a hydrostatic head of catholyte with respect to anolyte of 4 inches; and it should be great enough so that the overall cell voltage from anode to cathode is not more than 0.3 volt greater than in a comparable cell equipped with a cotton duck diaphragm weighing substantially 21 ounces per square yard.

In normal commercial operations, we prefer to employ a diaphragm having a permeability such that the flow of catholyte therethrough is about 22 cubic centimeters per square foot per minute under a hydrostatic head of catholyte with respect to anolyte in the range from  $\frac{3}{4}$  to  $1\frac{1}{2}$  inches.

The electrolyte employed in the electrolytic manganese process generally is saturated, or nearly so, with calcium sulfate, and this salt tends to crystallize in the pores of

the diaphragm fabric, particularly on the anode-facing side thereof where the electrolyte is strongly acidic. The accumulation of calcium sulfate (and other compounds as well) on and in the diaphragm material reduces its permeability. Consequently, after a diaphragm has been in service for a substantial period of time, generally from about six to eight weeks, the permeability of the diaphragm has become reduced to the point where it no longer functions satisfactorily. As stated above, cleaning and reusing the cotton diaphragms heretofore employed, after they have become thus plugged with salts, is quite impractical. It has therefore been customary to remove such diaphragms from the cell and replace them with new diaphragms. However, cleaning and reusing diaphragms of the invention, woven from fabrics of the above-specified synthetic fibers, is not only possible but is necessary in order to secure the full benefits of the invention. The fabrics used for making diaphragms in accordance with the invention are more costly than cotton, and it is only by making repeated use of each diaphragm, over a considerable number of cell cycles, that the important economies which the invention contemplates are realized.

In accordance with the invention, therefore, the new diaphragms are cleaned to remove the accumulation of salts after they have been in use for six to eight weeks, and they are then reused. This cycle of use for six to eight weeks followed by cleaning preparatory to further use may in accordance with the invention be repeated many times. Hence, although the initial cost of diaphragms made in accordance with the invention may be substantially higher than for cotton diaphragms, the ultimate cost is markedly less. Indeed, on the basis of our experience to date with operations carried out in accordance with the invention, it is conservative to state that approximately four-fifths of the cost for diaphragms can be saved by using diaphragms of the character herein specified and repeatedly cleaning them, as compared with using cotton duck diaphragms and replacing them after each cycle of use, as has heretofore been customary. In the case of the plant hereinbefore mentioned, in which the cost for cotton diaphragms in accordance with heretofore customary practice would be approximately \$25,000 per year, the saving effected in accordance with the invention may amount to four-fifths of this total, or \$20,000 per year.

Various procedures may be employed to clean the diaphragms in carrying out the method of this invention. In general, however, the cleaning operation involves the step of supporting the diaphragm in a cleaning tank and maintaining fresh water under slight pressure in contact with the cathode-facing surface thereof until the calcium sulfate deposits are loosened. The water pressure required is low, being only that necessary to keep the anode-facing surface of the diaphragm wet (preferably dripping wet) by seepage of water through the diaphragm. The cleaning method can be carried out by suitably supporting the diaphragm assemblies and filling them with water, or immersing them in a tank of water, whichever may be required to apply water to the cathode-facing surface. The hydrostatic head of the water in the diaphragm or in the cleaning tank, acting on the diaphragm, provides all the pressure that is necessary for the requisite seepage of water through the diaphragm. In the course of a few hours to a day or so, the fresh water seeping through the diaphragm dissolves enough of the calcium sulfate crystals where they penetrate the meshes of the fabric so that the whole deposit sloughs off or can easily be washed off.

The following examples illustrate the manner in which the invention is carried out:

#### Example I

A diaphragm was prepared using a heavy tightly woven fabric composed of fibers sold under the trade name

"Orlon" and composed essentially of polyacrylonitrile, a linear homopolymer with head-to-tail linkage of acrylonitrile, having substantially the formula  $[-\text{CH}_2\text{CH}(\text{CN})-]_n$ , in which  $n$  is an integer generally approximating 1500 but which, for a small proportion of the polymer, has other values extending as low as 350 and as high as 2200, the average molecular weight of the polymer being about 80,000 and the individual polymeric constituents having molecular weights in the range from about 19,000 to about 110,000. The fabric was woven from 5-ply 80 filament 200 denier filling strands and 10-ply 80 filament 200 denier warp strands, using 75 warp strands and 23 filling strands per linear inch. The fabric weighed about 18.5 ounces per square yard. The diaphragm was mounted in a conventional electrolytic manganese cell, where it was exposed on one side to an acidic anolyte having a pH generally in the range of 0.9 to 1.2 and containing generally from 125 to 140 grams per liter of ammonium sulfate and about 15 grams per liter of manganese (as manganeseous sulfate), and on the other side to an alkaline catholyte having a pH of about 8 to 9 and containing approximately the same amount of ammonium sulfate as the anolyte and about 35 grams per liter of manganese. The temperature of both anolyte and catholyte was in general maintained in the range from 35 to 45° C. Electrolytic manganese was deposited on the cathode immersed in the catholyte, by passing a direct electric current between the anode and cathode through the electrolytes and the diaphragm, over a period of about eight weeks. At the end of such period, a substantial crust of calcium sulfate crystals had collected on the anode-facing side of the diaphragm. The diaphragm assembly was removed from the cell, and was filled with fresh tap water. The fresh water seeped slowly through the diaphragm fabric to the outer surface thereof, which in service faced the anode, and on which the crust of calcium sulfate crystals had collected. After a period of about twenty-four hours, the crust of calcium sulfate crystals had become so loosened that it could easily be removed by hosing the outer surface of the diaphragm assembly with a stream of water. After further cleaning to remove manganese dioxide and other compounds that also had collected on it, the diaphragm assembly was returned to the electrolytic cell and was reused in the manner described above. The diaphragm showed no sign of deterioration, other than that incident to mechanical wear, over a period of many such cycles of use and cleaning.

Fabrics of fibers composed of "Teflon," a long-chain polymer of tetrafluoroethylene, also may be used in accordance with the invention. The molecule of this polymer consists of a long chain of relatively simple units having the formula  $-\text{CF}_2-$ . "Teflon" polymers are available in fiber form and can be woven into fabrics of the character described above, and having the properties required of diaphragms for use in accordance with this invention.

We claim:

1. The method of electrowinning manganese which comprises passing an electric current from an anode through an anolyte comprising an acidic manganeseous sulfate-ammonium sulfate solution, and through a catholyte comprising an alkaline manganese sulfate-ammonium sulfate solution to a cathode, characterized in that the anolyte and catholyte are separated by a closely woven permeable fabric diaphragm having a maximum permeability measured by the flow of catholyte therethrough into the anolyte of not more than about 25 cubic centimeters per square foot per minute under a hydrostatic head of catholyte with respect to anolyte of  $\frac{1}{2}$  inch, said diaphragm being capable of resisting physical deformation and change in its permeability characteristic during prolonged exposure to the electrolytes, and being woven of fibers of a linear homopolymer of a compound from the

group consisting of acrylonitrile and polytetrafluoroethylene.

2. The method according to claim 1, in which calcium is present in the anolyte, characterized in that the diaphragm is periodically withdrawn from the electrolytic operation, deposits of calcium sulfate are removed from the anode-facing surfaces thereof by supporting said diaphragm in a cleaning tank and maintaining fresh water under slight pressure in contact with the cathode-facing surface thereof until said deposits are loosened, the water pressure on the cathode-facing surface of the diaphragm being only sufficient to keep the anode-facing surface of the diaphragm wet by seepage of water through the diaphragm, and the cleaned diaphragm is returned to the electrolytic operation for further use therein.

3. The method of electrowinning manganese which comprises passing an electric current from an anode through an anolyte comprising an acidic manganeseous sulfate-ammonium sulfate solution and through a catholyte comprising an alkaline manganese sulfate-ammonium sulfate solution to a cathode, said anolyte and said catholyte being substantially saturated with dissolved calcium sulfate, the anolyte and catholyte being separated by a closely woven permeable fabric diaphragm initially having a permeability, as measured by the flow of catholyte therethrough into the anolyte, in the range from a maximum of about 25 cubic centimeters per square foot per minute under a hydrostatic head of catholyte with respect to anolyte of  $\frac{1}{2}$  inch to a minimum of about 20 cubic centimeters per square foot per minute under a hydrostatic head of catholyte with respect to anolyte of 4 inches, said diaphragm being capable of resisting physical deformation and change in its permeability characteristics during prolonged exposure to the anolyte and catholyte and being woven of fibers of a linear homopolymer of a compound from the group consisting of acrylonitrile and polytetrafluoroethylene, continuously adding electrolyte high in dissolved manganese to the catholyte and continuously withdrawing anolyte, continuing the electrolytic operation until a substantial crust of precipitated calcium sulfate has collected on a face of the diaphragm, withdrawing the diaphragm from the electrolytic operation, introducing fresh water under slight pressure into contact with the face of said diaphragm opposite that on which said calcium sulfate deposit has mostly collected, the water pressure being only sufficient to cause sufficient seepage of water through the diaphragm to keep dripping wet the surface on which the calcium sulfate deposit has mainly formed, maintaining the fresh water in contact with the diaphragm until the calcium sulfate deposit has loosened, removing the loosened deposit from the diaphragm, and returning the cleaned diaphragm to the electrolytic operation for reuse.

4. In a process for electrowinning manganese, in which an electric current is passed from an anode through an acidic manganese-bearing anolyte and an alkaline manganese-bearing catholyte to a cathode and in which the anolyte and catholyte are separated by a permeable diaphragm, the improvement which comprises employing as the diaphragm material a closely woven permeable fabric capable of resisting deformation with consequent change in permeability over a prolonged period of contact with said electrolytes, said diaphragm being woven of fibers consisting essentially of linear homopolymers of acrylonitrile having an average molecular weight of about 80,000, with individual polymeric constituents having molecular weights in the range from 19,000 to 110,000, said diaphragm having a permeability measured by the flow of catholyte therethrough into the anolyte of about 22 cubic centimeters per square foot per minute under a hydrostatic head of catholyte with respect to anolyte in the range from  $\frac{3}{4}$  to  $1\frac{1}{2}$  inches.

5. In a process for electrowinning manganese, in which an electric current is passed from an anode through an acidic manganese-bearing anolyte and an alkaline manga-

nese-bearing catholyte to a cathode and in which the anolyte and catholyte are separated by a permeable diaphragm, the improvement which comprises employing as the diaphragm material a closely woven permeable fabric capable of resisting deformation with consequent change in permeability over a prolonged period of contact with said electrolytes, said diaphragm being woven of fibers consisting essentially of polytetrafluoroethylene, said diaphragm having a permeability measured by the flow of catholyte therethrough into the anolyte of about 22 cubic centimeters per square foot per minute under a hydrostatic head of catholyte with respect to anolyte in the range from  $\frac{3}{4}$  to  $1\frac{1}{2}$  inches.

## References Cited in the file of this patent

## UNITED STATES PATENTS

1,120,629 Salisbury Dec. 8, 1914

## FOREIGN PATENTS

667,528 Great Britain Mar. 5, 1952

## OTHER REFERENCES

10 Quig: "Rayon and Synthetic Textiles," vol. 30, No. 4, April, 1949, page 92.

Jacobs et al.: "Metal Industry," Dec. 8, 1944, pages 358, 359.